

## UNITED STATES PATENT OFFICE

2,668,100

## CORROSION INHIBITOR FOR LIQUID HYDROCARBONS

George W. Luvisi, Chicago, Ill., assignor to National Aluminate Corporation, Chicago, Ill., a corporation of Delaware

No Drawing. Application November 15, 1951,  
Serial No. 256,603

20 Claims. (Cl. 44—63)

1

This invention relates to hydrocarbon liquids, more particularly gasoline, diesel fuel oil and furnace oils containing a corrosion inhibitor, and to a method of inhibiting corrosion caused by the presence of water in such liquids.

In copending application, Serial No. 186,929, of which the present application is a continuation-in-part, there are disclosed compounds which can be described as carbocyclic monocarboxy acid salts of glyoxalidines. The said application also describes the employment of certain of these compounds as emulsifying agents for aromatic oils in water.

In accordance with the present invention it has been found that certain of these carbocyclic monocarboxy acid salts of glyoxalidines are effective as corrosion inhibitors in hydrocarbon liquids.

The carbocyclic monocarboxy acid salts of glyoxalidines with which the invention is particularly concerned have the following general formula



wherein R is a higher aliphatic hydrocarbon radical containing at least 8, preferably 13 to 17 carbon atoms, inclusive, in an acyclic chain, R' is hydrogen or a lower aliphatic group containing not more than 6 carbon atoms, Y is hydrogen or a lower aliphatic group containing not more than 6 carbon atoms, and Z is hydrogen or a lower alkyl group containing not more than 6 carbon atoms. These compounds may also be described generally as salicylic acid salts of glyoxalidines.

The preferred compounds employed for the purpose of the present invention are compounds of the class previously described which are viscous liquids or soft greases characterized by being soluble or dispersible in water. The preferred compounds are also preferably soluble in aromatic oils when tested in the manner herein described. All of the compounds are sufficiently soluble in the hydrocarbon liquids to be effective for the purpose of the invention. In this connection it may be noted that the quantities required for the purpose of the invention are relatively small and are preferably within the range of 25 to 100 parts of the glyoxalidine salicylic acid salt per million parts

2

of hydrocarbon liquid. Even in amounts as low as ten parts per million some of these compounds are effective in inhibiting sludge formation in certain types of heavier oils where the formation of sludge is a problem, for example, in burning oils such as are used in locomotives and in diesel fuel oils.

The salicylic acid salts are prepared by mixing glyoxalidines and salicylic acid in equimolecular proportions in the cold or by warming the two together at temperatures up to 100° C. for 5 to 15 minutes, with or without a catalyst. The glyoxalidines are made by well known procedures by reacting a fatty acid with an aliphatic polyamine with the elimination of water as described for example, in Wilson, U. S. 2,267,965, and Wilkes et al., U. S. 2,268,273.

The salicylic acid salts of glyoxalidines with which the invention is particularly concerned are those salicylic acid salts in which the glyoxalidine portion of the molecule is derived by reacting together one of the acids from the group consisting of lauric acid, myristic acid, palmitic acid, oleic acid and stearic acid with an aliphatic polyamine from the group consisting of aminoethylmethylethanolamine, diethylenetriamine, and triethylenetetramine. When the glyoxalidine is derived from aminoethylmethylethanolamine the resultant product contains a hydroxyethyl group in the 1-position. When the glyoxalidine is derived from diethylenetriamine the resultant product contains an aminoethyl group in the 1-position, and when the glyoxalidine is derived from triethylenetetramine the resultant product contains a (2-aminoethyl)-aminoethyl group in the 1-position.

The number of carbon atoms in the aliphatic hydrocarbon group in the 2-position is always one less than that in the aliphatic carboxylic acid from which the glyoxalidine is derived.

Specific examples of glyoxalidines that can be reacted with salicylic acid in preparing salts suitable for the purpose of the invention are: 1-(2-hydroxyethyl)-2-undecyl glyoxalidine, 1-(2-hydroxyethyl)-2-tridecyl glyoxalidine, 1-(2-hydroxyethyl)-2-pentadecyl glyoxalidine, 1-(2-hydroxyethyl)-2-heptadecyl glyoxalidine, 1-(2-hydroxyethyl)-2-heptadecyl glyoxalidine, 1-(2-aminoethyl)-2-undecyl glyoxalidine, 1-(2-aminoethyl)-2-tridecyl glyoxalidine, 1-(2-aminoethyl)-2-pentadecyl glyoxalidine, 1-(2-aminoethyl)-2-heptadecyl glyoxalidine, 1-(2-aminoethyl)-2-undecyl glyoxalidine, 1-(2-aminoethyl)-2-tridecyl glyoxalidine, 1-(2-aminoethyl)-2-pentadecyl glyoxalidine, 1-(2-aminoethyl)-2-heptadecyl glyoxalidine, 1-(2-aminoethyl)-2-undecyl glyoxalidine, 1-(2-aminoethyl)-2-tridecyl glyoxalidine, 1-(2-aminoethyl)-2-pentadecyl glyoxalidine, 1-(2-aminoethyl)-2-heptadecyl glyoxalidine, 1-(2-aminoethyl)-2-undecyl glyoxalidine, 1-(2-aminoethyl)-2-tridecyl glyoxalidine, 1-

[(2-aminoethyl)-aminoethyl]-2-pentadecyl glyoxalidine, 1-[(2-aminoethyl)-aminoethyl]-2-heptadecyl glyoxalidine, 1-[(2-aminoethyl)-aminoethyl]-2-heptadecyl glyoxalidine, 4-methyl-2-tridecyl glyoxalidine, 4-methyl-2-pentadecyl glyoxalidine, 4-methyl-2-heptadecyl glyoxalidine 4-methyl-2-heptadecenyl glyoxalidine.

The following table contains some of the properties of glyoxalidine salicylates that have been employed in accordance with the invention:

| Reactants                                                    | Weight Ratio | Description                             | Solubility in Water                             | Solubility in Aromatic Oil |
|--------------------------------------------------------------|--------------|-----------------------------------------|-------------------------------------------------|----------------------------|
| 1-(2-hydroxyethyl)-2-heptadecenyl glyoxalidine.              | 3.5          | homogeneous viscous liquid.             | slightly cloudy; foams copiously; very viscous. | soluble.                   |
| Salicylic acid.                                              | 1.38         |                                         | clear gelatinous solution; fairly heavy foam.   | Do.                        |
| 2-heptadecenyl-4-methyl glyoxalidine.                        | 3.2          | homogeneous yellow viscous liquid.      | clear gelatinous solution; very heavy foam.     | insoluble.                 |
| Salicylic acid.                                              | 1.38         |                                         | turbid solution; fairly heavy foam.             | Do.                        |
| 1-[2-(2-aminoethyl)-aminoethyl]-2-heptadecenyl-glyoxalidine. | 3.93         | homogeneous deep yellow viscous liquid. | clear solution; extremely heavy foam.           | Do.                        |
| Salicylic acid.                                              | 1.38         |                                         | hazy solution; quite viscous; lots of foam.     | soluble.                   |
| 2-heptadecenyl-4-methyl glyoxalidine.                        | 3.2          | clear amber viscous liquid.             |                                                 |                            |
| Salicylic acid.                                              | 2.76         |                                         |                                                 |                            |
| 1-[2-(aminoethyl)-aminoethyl]-2-heptadecenyl glyoxalidine.   | 3.93         | cloudy amber tafty-like liquid.         |                                                 |                            |
| Salicylic acid.                                              | 2.76         |                                         |                                                 |                            |
| 1-(2-hydroxyethyl)-2-heptadecenyl glyoxalidine.              | 3.5          | viscous oil.                            |                                                 |                            |
| 2,6-dichloro-salicylic acid.                                 | 2.07         |                                         |                                                 |                            |

The solubility test of the glyoxalidine salt in water was conducted by adding one drop of the salt to 10 ml. of water and agitating and observing the resulting solution.

The solubility of the glyoxalidine salt in oil was determined by adding one drop of the salt to 10 ml. of an aromatic oil such as the catalytically cracked product marketed by Shell Oil Company under the trade name of Shell's medium aromatic oil with a boiling range of 430° F. to 620° F. and a flash point of 225° F. (Cleveland open cup).

The corrosion inhibiting properties of these new compounds will be further illustrated by the following examples.

#### Example I

The glyoxalidine salicylic acid salt was prepared for use as a 10% by weight concentrate in a suitable solvent, for example, xylene and/or naphtha.

The test specimens were hot rolled mild steel rods  $\frac{1}{4} \times 2\frac{3}{4}$ " of which a  $2\frac{1}{4}$ " length was polished with #3/0 emery cloth.

The test medium, for example, gasoline, was placed in a 25 x 150 mm. screw cap tube. To 40 ml. of the test medium were added first the inhibitor solution previously described and after mild agitation 10% by volume of distilled water which had been equilibrated with air. The capped tube was then mechanically agitated at room temperature (75° F.) for six hours by end over end tumbling.

The test solution was then transferred to a numbered 25 x 150 mm. test tube and the water and hydrocarbon phases were permitted to separate. The test specimen was inserted in the tube so that a part was exposed to the lower phase (water) without contacting any part of the container. The tube was not disturbed for the 72-hour test duration.

Other tests were set up as described above with selected materials in which 1% water instead of 10% was used.

After completion of the test the specimen was removed, rinsed with acetone and air dried. It

was then evaluated on the extent of visible corrosion. Each test was made in duplicate. If both specimens were not visibly corroded the material was classed as effective and if both appeared to be corroded the material was called ineffective. Wherever one of the pairs was uncorroded and the other corroded the test was repeated. If, after retesting, either specimen was corroded the material was judged to be ineffective at the tested concentration. This criterion is identical with that used in ASTM D665-49T.

The inhibitor materials were generally tested at 50 p. p. m. (parts per million) of test medium with the concentration being varied whenever further testing was warranted.

The salicylic acid salt of 1-(2-hydroxyethyl)-2-heptadecenyl glyoxalidine when tested under the foregoing conditions in Standard Red Crown gasoline was effective in inhibiting corrosion in three tests at a concentration of 25 p. p. m., in two tests at a concentration of 40 p. p. m. and in one test at a concentration of 50 p. p. m. At concentrations of 5 and 10 p. p. m. with this material the test specimens showed slight corrosion. At concentrations of 15 and 20 p. p. m. six test results showed no corrosion to vary slight corrosion. In all of these tests the test medium contained 10% distilled water.

Similar tests conducted with the 1-(2-hydroxyethyl)-2-heptadecenyl glyoxalidine salicylic acid salt in the same test medium containing 1% by volume of distilled water gave results similar to those obtained with 10% by volume of distilled water.

All of the foregoing tests were made at room temperatures of approximately 75° F. The water saturated gasoline did not corrode the steel specimens during a test period of six weeks.

#### Example II

The testing procedure was the same as that described in Example I using Standard Red Crown gasoline and 10% distilled water in the medium. 1-(2-aminoethyl)-2-tridecyl glyoxalidine salicylic acid salt was effective in inhibiting corrosion at concentrations of 25 p. p. m. and 50 p. p. m. of test medium. At a concentration of 10 p. p. m. the corrosion was slight to moderate at the end of the test period of 72 hours.

#### Example III

Using the test procedure described in Example I with Standard Red Crown gasoline and 10% by volume of distilled water in the test medium the 1-(2-aminoethyl)-2-pentadecyl glyoxalidine salicylic acid salt gave substantially the same results as those described in Example II.

*Example IV*

Using the test procedure described in Example I with Standard Red Crown gasoline and 10% by volume of distilled water in the test medium the 4-methyl-2-heptadecenyl glyoxalidine salicylic acid salt produced no corrosion to very slight corrosion at a concentration of 25 p. p. m. in the test medium and no corrosion at a concentration of 50 p. p. m. in the test medium at the end of the 72 hour test period. Concentrations of 5 and 10 p. p. m., respectively produced moderate corrosion.

*Example V*

Using the test procedure described in Example I with Standard Red Crown gasoline and 10% by volume distilled water in the test medium the 1 - [2 - (2 - aminoethyl) - aminoethyl] - 2-heptadecenyl glyoxalidine salicylic acid salt was effective in preventing corrosion at a concentration of 50 p. p. m. in the test medium. At a concentration of 25 p. p. m. the test specimens showed slight corrosion at the end of the 72-hour test.

*Example VI*

The test procedure was the same as that described in Example I except that Stanolind diesel fuel oil was used in place of the Standard Red Crown gasoline and the quantity of water added to the test medium was 10% by volume. The salicylic acid salt described in Example I was completely effective in preventing corrosion in the diesel fuel oil samples at a concentration of 100 p. p. m. in the test medium.

*Example VII*

The test procedure was the same as that used in Example I except that Stanolex furnace oil containing 10% by volume distilled water was used as the test medium. The salicylic acid salt described in Example I was effective as a corrosion inhibitor at 50 p. p. m. in the test medium. At a concentration of 25 p. p. m. very slight corrosion of the test specimens was observed at the end of the 72-hour test period.

*Example VIII*

The 1-(2 - hydroxyethyl) - 2(3,5,5 - trimethylpentyl) glyoxalidine salicylic acid salt was prepared by adding 39.5 grams of 3,5,5-trimethylhexanoic acid and 26 grams of aminoethyl-ethanolamine to 220 cc. of xylene and heating at a temperature of 161° C. to 169° C. for approximately 20 hours with the elimination of 8.9 cc. of water. The xylene was removed by distillation and the residue was distilled at 1 to 2 mm. pressure at a temperature of 169° C. to 190° C. The resultant glyoxalidine was a greenish yellow viscous liquid. Equimolecular proportions of this product and salicylic acid were reacted by heating on a steam bath for 15 minutes to produce the salicylic acid salt.

The resultant salt was found to be insoluble in Indocene 90 (a Standard Oil of Indiana petroleum fraction high in aromatic compounds and naphthenes) and therefore was dissolved as a 10% solution in the monobutyl ether of diethylene glycol. This solution was added to Stanolind diesel fuel oil and testing according to the procedure described in Example I. At a concentration of 100 p. p. m. of the salicylic acid salt effective corrosion inhibition was obtained in the water phase. In the oil phase there was no corrosion of the test specimens at concentrations

as low as 10 p. p. m. A comparative test with the solvent material (the monobutyl ether of diethylene glycol) at 900 p. p. m. showed that the solvent did not provide any protection in the water phase even at this relatively large concentration.

Since the effective corrosion inhibiting ingredient is employed in accordance with the invention in very small amounts, it is desirable to prepare it in the form of a solution containing about 5 to 15% of the effective ingredient, the remainder being a suitable solvent. Any solvent which is miscible with the corrosion inhibiting ingredient and the medium to which it is to be added can be employed for the purpose of the invention. As an illustration, where the corrosion inhibiting ingredient is to be added to gasoline a suitable concentrate has the following composition:

|                                                                    | Weight per cent |
|--------------------------------------------------------------------|-----------------|
| 1-(2-hydroxyethyl)-2-heptadecenyl glyoxalidine salicylic acid salt | 12              |
| Naphtha (flash point 80° F. to 105° F.)                            | 68              |
| Xylene                                                             | 20              |

Similarly, other compositions can be prepared using as a solvent either naphtha alone or xylene alone or other suitable solvents such as diethylene glycol monobutyl ether and mixtures thereof with naphtha and/or xylene.

Where the concentrate is to be added to a diesel fuel oil or a furnace oil the solvent should have characteristics compatible with those of the diesel fuel oil or the furnace oil. In some cases the diesel fuel oil or the furnace oil has been used as the solvent in the concentrate. Indocene 90 has been employed very satisfactorily as a solvent for the salicylic acid salt in concentrates used as additives for furnace oils and diesel fuel oil except in those instances where the salicylic acid salt is insoluble in this solvent as in Example VIII.

The dosage required for effective corrosion inhibition is very often different in gasoline and heavier hydrocarbon liquids such as diesel oil and furnace oil. In general, it is desired for the purpose of the invention that the corrosion inhibitor be effective at concentrations of not more than 100 parts per million parts by weight of the hydrocarbon liquid. Especially in gasoline the introduction of large amounts of the corrosion inhibitor could have very adverse effects, such as gum formation. In actual tests using in one case a composition composed of 12% of the salicylate described in Example I and 88% of Indocene 90 and in another case a composition composed of 12% of the salicylate described in Example I, 68% of Stanisol Stoddard solvent and 20% xylene there was only a slight increase in gum formation in the first instance and a decrease in the second instance at concentrations of 25 p. p. m. and 12.5 p. p. m. of the salicylates, respectively.

The best results in the prevention of corrosion in gasoline were obtained with the glyoxalidine salicylic acid salt described in Example I and purified samples thereof. This salt is insoluble in the monobutyl ether of diethylene glycol, soluble in 100% ethanol, soluble in Indocene 90, soluble in 99% isopropanol, soluble in xylene, insoluble in Stanisol Stoddard solvent and insoluble in virgin gas oil.

In general, the greatest corrosion produced by compositions containing hydrocarbon liquids and water appears to occur in the water phase where

there is a separation of the water. Many closely related materials were tested and found to be ineffective at concentrations where the compositions of the present invention are effective, for example at 50 p. p. m. In gasoline the acetate and benzoate salts of the glyoxalidines containing an aliphatic hydrocarbon chain having eight or more carbon atoms in the 2-position were ineffective. At the same concentration in gasoline the salicylate of the glyoxalidine derived by reacting diethylenetriamine with ethylhexanoic acid and which contains a seven carbon atom alkyl group in the 2-position was ineffective. Likewise, at the same concentration in gasoline the glyoxalidines derived by reacting diethylenetriamine with lauric acid; diethylenetriamine with myristic acid; diethylenetriamine with palmitic acid; triethylenetetramine with oleic acid; aminoethylethanolamine with oleic acid; and diethylenetriamine with nonoic acid were ineffective in inhibiting corrosion under the test conditions previously described.

The invention is hereby claimed as follows:

1. A hydrocarbon liquid containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, the carbon atom in the 5-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

2. Gasoline containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, the carbon atom in the 5-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

3. A diesel fuel oil containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, the carbon atom in the 5-position is linked to a member from the group consisting of hydrogen and lower aliphatic groups containing not more than 6 carbon atoms, there being at least one hydrogen atom on each of the carbon atoms in the 4- and 5-positions, and the

nitrogen atom in the 1-position is linked to a member from the group consisting of hydrogen and lower aliphatic groups containing not more than 6 carbon atoms, there being at least one hydrogen atom attached to said nitrogen atom.

4. A furnace fuel oil containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, the carbon atom in the 5-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

5. A hydrocarbon liquid containing a corrosion inhibiting amount of a salicylic acid salt of a glyoxalidine having the following general formula



wherein R is a higher aliphatic group containing 13 to 17 carbon atoms, inclusive, in an acyclic chain, R' is a member from the group consisting of hydrogen and lower aliphatic groups containing not more than 6 carbon atoms, Y is a member from the group consisting of hydrogen and lower aliphatic groups containing not more than 6 carbon atoms, and Z is a member from the group consisting of hydrogen and lower alkyl groups containing not more than 6 carbon atoms.

6. Gasoline containing a corrosion inhibiting amount of a salicylic acid salt of a glyoxalidine wherein the carbon atom in the 2-position is linked to a higher aliphatic hydrocarbon group containing 13 to 17 carbon atoms, inclusive, in an acyclic chain, the carbon atoms in the 4- and 5-positions are linked to a member from the group consisting of hydrogen and lower aliphatic groups containing not more than 6 carbon atoms and the nitrogen atom in the 1-position is linked to a 2-hydroxyethyl group.

7. Gasoline containing a corrosion inhibiting amount of a salicylic acid salt of a glyoxalidine wherein the carbon atom in the 2-position is linked to a higher aliphatic hydrocarbon group containing 13 to 17 carbon atoms, inclusive, in an acyclic chain, the carbon atoms in the 4- and 5-positions are linked to a member from the group consisting of hydrogen and lower aliphatic groups containing not more than 6 carbon atoms and the nitrogen atom in the 1-position is linked to a 2-aminoethyl group.

8. Gasoline containing a corrosion inhibiting amount of a salicylic acid salt of a glyoxalidine wherein the carbon atom in the 2-position is linked to a higher aliphatic hydrocarbon group containing 13 to 17 carbon atoms, inclusive, in an acyclic chain, the carbon atoms in the 4- and

5-positions are linked to a member from the group consisting of hydrogen and lower aliphatic groups containing not more than 6 carbon atoms and the nitrogen atom in the 1-position is linked to a 2-(aminoethyl)-aminoethyl group.

9. A hydrocarbon liquid containing a corrosion inhibiting amount of 1-(2-hydroxy-ethyl)-2-heptadecenyl glyoxalidine salicylic acid salt.

10. Gasoline containing about 20 to about 50 parts per million of 1-(2-hydroxy-ethyl)-2-heptadecenyl glyoxalidine salicylic acid salt.

11. A method of inhibiting corrosion of ferrous metals by hydrocarbon liquids containing water which comprises bringing said metals into contact with said liquids containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

12. A method of inhibiting corrosion of ferrous metals by gasoline contaminated with moisture which comprises bringing said metals into contact with said gasoline containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

13. A method of inhibiting corrosion of ferrous metals by a diesel fuel oil contaminated with moisture which comprises bringing said metals into contact with said diesel fuel oil containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

taining not more than 6 carbon atoms, there being at least one hydrogen atom attached to said nitrogen atom.

14. A method of inhibiting corrosion of ferrous metals by a furnace fuel oil contaminated with moisture which comprises bringing said metals into contact with said furnace fuel oil containing a corrosion inhibiting amount of a salicylic acid salt of a glyoxalidine wherein the carbon atom in the 2-position is linked to a higher aliphatic hydrocarbon group containing at least 8 carbon atoms, the carbon atom in the 4-position is linked to a member from the group consisting of hydrogen and lower aliphatic groups containing not more than 6 carbon atoms, there being at least one hydrogen atom on each of the carbon atoms in the 4- and 5-positions, and the nitrogen atom in the 1-position is linked to a member from the group consisting of hydrogen and lower aliphatic groups containing not more than 6 carbon atoms, there being at least one hydrogen atom attached to said nitrogen atom.

15. A method of inhibiting corrosion of ferrous metals by a hydrocarbon liquid containing water which comprises bringing said metals into contact with said liquid containing a corrosion inhibiting amount of a salicylic acid salt of a glyoxalidine having the following general formula



wherein R is a higher aliphatic group containing 13 to 17 carbon atoms, inclusive, in an acyclic chain, R' is a member from the group consisting of hydrogen and lower aliphatic groups containing not more than 6 carbon atoms, Y is a member from the group consisting of hydrogen and lower aliphatic groups containing not more than 6 carbon atoms, and Z is a member from the group consisting of hydrogen and lower alkyl groups containing not more than 6 carbon atoms.

16. A method of inhibiting corrosion of ferrous metals by gasoline contaminated with moisture which comprises bringing said metals into contact with said gasoline containing a corrosion inhibiting amount of a salicylic acid salt of a glyoxalidine wherein the carbon atom in the 2-position is linked to a higher aliphatic hydrocarbon group containing 13 to 17 carbon atoms, inclusive, in an acyclic chain, the carbon atoms in the 4- and 5-positions are linked to a member from the group consisting of hydrogen and lower aliphatic groups containing not more than 6 carbon atoms and the nitrogen atom in the 1-position is linked to a 2-hydroxyethyl group.

17. A method of inhibiting corrosion of ferrous metals by gasoline contaminated with moisture which comprises bringing said metals into contact with said gasoline containing a corrosion inhibiting amount of a salicylic acid salt of a glyoxalidine wherein the carbon atom in the 2-position is linked to a higher aliphatic hydrocarbon group containing 13 to 17 carbon atoms, inclusive, in an acyclic chain, the carbon atoms in the 4- and 5-positions are linked to a member from the

11

group consisting of hydrogen and lower aliphatic groups containing not more than 6 carbon atoms and the nitrogen atom in the 1-position is linked to a 2-aminoethyl group.

18. A method of inhibiting corrosion of ferrous metals by gasoline contaminated with moisture which comprises bringing said metals into contact with said gasoline containing a corrosion inhibiting amount of a salicylic acid salt of a glyoxalidine wherein the carbon atom in the 2-position is linked to a higher aliphatic hydrocarbon group containing 13 to 17 carbon atoms inclusive in an acyclic chain, the carbon atoms in the 4- and 5-positions are linked to a member from the group consisting of hydrogen and lower aliphatic groups containing not more than 6 carbon atoms and the nitrogen atom in the 1-position is linked to a 2-(aminoethyl)-aminoethyl group.

19. A method of inhibiting corrosion of ferrous

5

10  
15

12

metals by a hydrocarbon liquid containing water which comprises bringing said metals into contact with said liquid containing a corrosion inhibiting amount of 1-(2-hydroxy-ethyl)-2-heptadecenyl glyoxalidine salicylic acid salt.

20. A method of inhibiting corrosion of ferrous metals by gasoline contaminated with water which comprises bringing said metals into contact with said gasoline containing about 20 to about 50 parts per million of 1-(2-hydroxy-ethyl)-2-heptadecenyl glyoxalidine salicylic acid salt.

GEORGE W. LUVISI.

## References Cited in the file of this patent

## UNITED STATES PATENTS

| Number    | Name  | Date         |
|-----------|-------|--------------|
| 2,553,183 | Caron | May 15, 1951 |